

## UNITED STATES PATENT OFFICE

ARCHIBALD JOHN HALL, OF CONGLETON, ENGLAND, ASSIGNOR TO THE SILVER SPRINGS BLEACHING & DYEING COMPANY LIMITED, OF TIMBERSBROOK, CONGLETON, ENGLAND

## PROCESS IN WHICH VISCOSE SILK IS SUBJECTED TO THE ACTION OF CAUSTIC ALKALIS

No Drawing. Application filed June 23, 1928, Serial No. 287,894, and in Great Britain July 9, 1927.

This invention relates to processes for the treatment with a caustic alkali of textile materials such as yarns and fabrics, composed wholly or partly of desulfurized viscose.

5 It is known that when desulfurized viscose silk is exposed to the action of solutions of caustic soda it loses its soft feel and becomes harsh and brittle, this deleterious effect being generally greater as the concentration of 10 the caustic soda is increased. In consequence of this behaviour of viscose silk towards caustic soda it has been found very difficult to treat yarns and fabrics composed wholly or partly of desulfurized viscose with processes 15 which require the use of caustic soda. One of such processes which is frequently desired to apply to cotton fabrics or yarns containing desulfurized viscose is the process of mercerization in which process caustic soda is 20 employed as the mercerizing agent.

We have now discovered that the behaviour of desulfurized viscose silk towards solutions of caustic potash is quite different from its behaviour under similar circumstances towards caustic soda, although this difference could not be foreseen without experiment. In particular we have found that desulfurized viscose silk is much less affected by caustic potash than by caustic soda and 30 we have applied this discovery to various processes for treatment of yarns and fabrics composed wholly or partly of viscose silk and particularly to the mercerization of cotton materials containing desulfurized viscose silk, although it is to be understood that it may also be applied in the treatment with a 35 caustic alkali of materials containing other fibres such as linen and which also contain desulfurized viscose.

40 Our investigations of the action of caustic potash on desulfurized viscose silk show that such action is influenced by the duration of the treatment, and also by the concentration and temperature of the solution of caustic 45 potash employed. In general it has been observed that caustic potash reduces the softness of handle of desulfurized viscose silk to a greater extent as the temperature of the caustic potash is decreased. It is therefore 50 preferred to use for purposes of merceriza-

tion solutions of caustic potash at 15°-50° C., and even higher temperatures. The deleterious action of caustic potash on the handle of desulfurized viscose silk also increases with the duration of treatment, so that it is 55 preferred to carry out the operation of mercerization in the shortest time which allows the desired mercerization effects to be obtained. Although solutions of caustic potash of 70° Tw. appear to exert the maximum 60 deleterious action on desulfurized viscose silk, the influence of concentration is small.

In applying this invention to the mercerization of cotton materials containing desulfurized viscose silk we adjust the conditions 65 of duration, concentration, and temperature such that the desulfurized viscose silk is not deleteriously effected whilst the cotton is satisfactorily mercerized.

The following is an example of the manner 70 in which this invention is applied to the mercerization of cotton fabric containing desulfurized viscose silk which may be present in warp or weft or both, it being clearly understood that this invention is not limited to the 75 conditions stated therein.

*Example*

Cotton fabric consisting of a cotton warp and a desulfurized viscose weft is successively impregnated with a solution of caustic potash of 60° Tw. at 30° C., stretched to the desired width, washed with cold or hot water while in the stretched condition, passed through a bath of dilute sulphuric acid, and afterwards thoroughly washed and dried. The duration of the processes of impregnation with caustic potash, stretching, and washing up to the commencement of acidification occupy together about 80 seconds. In 80 the resulting fabric, the cotton is well mercerized whilst the desulfurized viscose silk has retained its original strength, lustre and softness of handle.

What I claim as my invention and desire 85 to protect by Letters Patent is:—

1. A process for mercerizing textile fabrics containing desulfurized viscose silk consisting in treating such materials with a solution of caustic potash under conditions of 100

time, temperature, and concentration which are adjusted so that the cotton is mercerized to the desired degree whilst the desulfurized viscose silk is not deleteriously affected.

5 2. A process for mercerizing textile fabrics containing desulfurized viscose silk consisting in treating such materials with a solution of caustic potash so that the cotton is mercerized to the desired degree whilst the desulfurized viscose silk is not deleteriously affected and finally subjecting the material to tension.

10 3. A process for mercerizing textile fabrics containing desulfurized viscose silk consisting in impregnating the material with a solution of caustic potash of 55° to 60° Tw. at a temperature of over 15° C., stretching the material to the desired width, washing it with water while in the stretched condition, 15 passing through a bath of dilute sulphuric acid and finally washing and drying.

20 In testimony whereof I have hereunto set my hand.

ARCHIBALD JOHN HALL.